

## UNITED STATES PATENT OFFICE.

FRITZ NETZ, OF MARYSVILLE, KANSAS.

## COMPOUND FOR TREATING STEEL.

No Drawing.

Application filed August 5, 1924. Serial No. 730,245.

To all whom it may concern:

Be it known that I, FRITZ NETZ, a citizen of the United States, residing at Marysville, in the county of Marshall and State of 5 Kansas, have invented certain new and useful Improvements in Compound for Treating Steel, of which the following is a specification.

This invention relates to a compound for 10 treating steel.

The primary object of this invention is to provide, in a manner as hereinafter set forth, a compound for treating steel to impart thereto a hardness without causing the same 15 to become brittle, in other words, to harden the steel without causing it to lose its toughness or flexibility, so that the metal will not chip or break.

A further important object of this invention 20 is to provide, in a manner as hereinafter set forth, a compound for hardening steel, the use of which requires no complicated procedure, the method of operation being to simply plunge the article to be treated 25 into the compound, after heating to the proper temperature, and allowing the same to cool therein.

Although the compound can be used for 30 treating any article desired, it has been found to be especially fine for tempering tools such as picks, axes, cold chisels, plow shares and lathe tools.

The composition embodying this invention 35 comprises, soft water, laundry soap, brown sugar, old style cut tobacco, potassium cyanide (powdered) and beef tallow, all intimately mixed and when ready for use occurring as a plastic or semi-solid mass.

Experiment has shown that the best 40 results are obtained when the above named ingredients are combined in approximately the following proportions:

Soft water, 5 lbs.; laundry soap, 6 bars (30 ozs.); brown sugar, 4 ozs.; old style cut tobacco, 2½ ozs.; potassium cyanide (powdered), 1½ ozs.; beef tallow, 3 lbs.

The above ingredients are mixed in the following manner:—The soap is dissolved in a portion of the water while the tobacco

is well soaked in another heated portion of 50 the water, which is then added to the soap solution. The brown sugar, previously dissolved in another portion of the water, is then added together with the dissolved potassium cyanide. The tallow is melted 55 and added while hot to the mixture, which is then boiled for twenty minutes, with constant stirring.

The compound is then allowed to cool, 60 with frequent stirring to prevent separation of the ingredients, and when completely congealed a semi-solid plastic mass results.

Experiment has disclosed that the brown 65 sugar and tobacco cause the metal to have a toughness and hardness obtainable from no other substances. The potassium cyanide and beef tallow also harden the metal to a durable temper, while the soap and water give a proper body to the mixture, which prevents too rapid hardening of the steel, 70 thus avoiding brittleness.

When the mass has been cooled and set it 75 is ready for use without further preparation, and the article to be treated, after heating to the proper temperature, is plunged into the mass and allowed to cool therein, and as a result the article will be properly tempered, and if a cutting tool, it will be found to have an edge which will not break, nick 80 or become quickly dulled.

Having thus described my invention what I claim is:—

1. A metal treating compound of the character set forth, comprising a mixture of laundry soap, brown sugar, old style cut 85 tobacco, potassium cyanide, beef tallow and water, substantially as set forth.

2. A metal treating compound of the character set forth, comprising the following ingredients in approximately the following 90 proportions:—laundry soap 30 ounces, brown sugar 4 ounces, old style cut tobacco 2½ ounces, potassium cyanide (powdered) 1½ ounces, beef tallow 48 ounces and soft water 80 ounces.

In testimony whereof, I affix my signature hereto.

FRITZ NETZ.